

Feb. 26, 1924.

1,484,885

C. HAMBUECHEN

DEPOLARIZING COMPOSITION

Filed July 28, 1921



Inventor:  
Carl Hambuechen,  
748 Byrnes, Townsend  
& Brickenstein,  
Attorneys.

## UNITED STATES PATENT OFFICE.

CARL HAMBUECHEN, OF NEW YORK, N. Y., ASSIGNOR TO UNION CARBIDE AND CARBON RESEARCH LABORATORIES, INC., A CORPORATION OF NEW YORK.

## DEPOLARIZING COMPOSITION.

Application filed July 28, 1921. Serial No. 488,180.

To all whom it may concern:

Be it known that I, CARL HAMBUECHEN, a citizen of the United States, residing at New York, in the county of New York and State of New York, have invented certain new and useful Improvements in Depolarizing Compositions, of which the following is a specification.

This invention relates to depolarizers for electric cells and has particular reference to improvements in molded depolarizing mix compositions.

In dry cells of the type in which the depolarizer is molded about a carbon rod to form a "mix bobbin," it is usual to guard against the crumbling of the mix by coating the bobbin with an adhesive material or by wrapping it in a fabric. Adequate surface protection of this nature is essential, because jarring and softening by the electrolyte may otherwise result in partial disintegration of bobbins having the composition now standard. Particles so detached are likely to come into contact with the zinc electrode, causing harmful local action. I have discovered, further, that the current output of cells having mix bobbins of the type referred to is adversely affected by the jarring incidental to handling, shipping, and the like. Even where there is no apparent disintegration, the lack of adequate coherence within the mix bobbin may cause fissuring or other physical changes which increase resistance and lower depolarizing efficiency.

It is an object of my invention to provide a mix bobbin of increased stability, both with regard to surface erosion and to changes in internal structure which result in lowered amperage. This object is attained by bonding the particles of the mix composition with a fibrous material, such as asbestos, in a manner more fully described hereinafter.

The accompanying drawing illustrates one type of cell in which my invention finds advantageous application. In this drawing,

Fig. 1 is a vertical section through the cell, and

Fig. 2 is a perspective view of the bobbin.

Reference numeral 1 indicates a cylindrical zinc container electrode of ordinary type, 2 a carbon electrode, and 3 and 4 connecting wires. A depolarizing composition

5, containing a fibrous bonding agent, surrounds the carbon electrode 2. Paper caps 6 and 7 may be fitted over the ends of the depolarizer, as described in my Patent No. 1,375,632, issued April 19, 1921, but these are not essential for the success of the present invention. A disk 8, of cardboard or the like, encircles the carbon rod and lies adjacent the top of bobbin 5. Excitant paste 9 occupies all of the annular space between the depolarizer and the zinc container, except a small portion serving as an air chamber 10. A seal 11 closes the cell.

The mix bobbin 5 may be made up in the usual manner, except for the incorporation of the bonding material. I prefer to distribute somewhat less than 1% by weight of asbestos fiber throughout the depolarizing mix composition, but the proportion may be considerably varied according to the nature and degree of subdivision of the mix particles, the size and service requirements of the cell, or other conditions. As a specific illustration of one of the ways in which the invention may be advantageously used, about 1% by weight of asbestos fiber is intimately mixed with a depolarizer composition comprising finely divided pyrolusite and coke in approximately the ratio 2:1, prepared by being milled together as described in the application of W. R. Clymer, Serial No. 410,923, filed September 17, 1920. Either long or short fibered asbestos may be used, but the latter is preferable.

My invention is not limited to manganese dioxide and carbon compositions, but is applicable broadly to the preparation of bonded depolarizers from any suitable reducible substance. Other fibrous materials which are inert or have no harmful effect upon the cell may be substituted for asbestos. For example, good results are obtained by the use of cellulosic fibrous materials, such as wood pulp or the filaments of cotton or linen.

The permeability of the mix to electrolyte solution is increased by the presence of the fibrous material and the service characteristics of the cell are improved for this reason, as well as by the coherence due to the bonding of the mix particles.

Depolarizer compositions made up with a bonding agent as described may be tamped, molded to form mix bobbins, or otherwise suitably treated in preparation

for use in either dry or wet cells. Under ordinary conditions, wrapping or coating of mix bobbins containing the fibrous binder is unnecessary, but such additional protection may be provided if desired. Various substitutions with respect to the proportions, manipulations and uses specified by way of example above may be made within the scope of the appended claims.

10 1 claim:

1. A dry cell depolarizing composition comprising granular ingredients and containing a fibrous material serving as a binder.

15 2. The invention according to claim 1, in which the fibrous material is asbestos.

3. The invention according to claim 2, in which the asbestos is present in amount of about  $\frac{1}{2}\%$  by weight.

20 4. A dry cell depolarizing composition comprising a coherent body containing a fibrous material adapted to increase the stability of the body.

25 5. A permeable dry cell depolarizing composition comprising carbon and manganese dioxid, each in comminuted condition, and a fibrous material in admixture therewith and serving as a binder.

6. A dry cell comprising a metal container electrode, a carbon electrode and as- 30 sociated depolarizing mass therein, said mass comprising a fibrous binding ingredient.

7. A dry cell comprising a metal container electrode, a carbon electrode therein, 35 and a depolarizing mass associated with said carbon electrode and protected from disintegration only by a fibrous binding material incorporated in said mass.

8. Process of making a depolarizing composition for use in dry cells, comprising mixing comminuted substances capable of acting as a depolarizer with a fibrous material adapted to serve as a binder for such substances.

45 9. Process of making a depolarizing composition for use in dry cells, comprising mixing conductive carbon and manganese depolarizer, each in comminuted condition, with a fibrous material, and forming the 50 mixture into a coherent body in which the fibrous material serves as a binder.

In testimony whereof, I affix my signature.

CARL HAMBUECHEN.